

Aug. 10, 1954

I. J. NOVAK  
REFINEMENT OF ASBESTOS

2,685,825

Filed May 28, 1949

2 Sheets-Sheet 1



Inventor:  
Izador J. Novak  
By Lee J. Gary Atty.

Aug. 10, 1954

I. J. NOVAK  
REFINEMENT OF ASBESTOS

2,685,825

Filed May 28, 1949

2 Sheets-Sheet 2

FIG. 5.



FIG. 7.



FIG. 6.



Inventor:  
Izador J. Novak  
By Lee J. Gary Atty.

## UNITED STATES PATENT OFFICE

2,685,825

## REFINEMENT OF ASBESTOS

Izador J. Novak, Trumbull, Conn., assignor to  
Raybestos-Manhattan, Inc., Passaic, N. J., a  
corporation of New Jersey

Application May 28, 1949, Serial No. 96,062

1 Claim. (Cl. 92—20)

1

This invention relates to a novel method for refinement of asbestos without impairing the quality and fabricating properties of the asbestos fibers.

More particularly, the present invention relates to a novel method for removing associated impurities from chrysotile asbestos, such as serpentine fragments, magnetite inclusions, rock, pieces of wood, altered asbestos which is not amenable to fiberization, unopened asbestos bits of harsh yellow fiber (picrolite), and other unopened, unopenable or oversize bits or bundles of asbestos fiber.

It is known to remove concomitant impurities from asbestos by such methods as by subjecting mechanically fiberized material to vibratory screening; agitation by air blasts to separate heavy particles by gravity; flotation processes for separating mineral impurities; and the like. It is also known to refine cellulose fibers by such means as screening or centrifuging. However, it is not possible by prior known fiber refining or screening methods to prepare a mix of asbestos fibers, particularly asbestos fibers of spinning grade length, dry or wet, which is free or substantially free of oversized pieces of foreign matter or asbestos fiber matter above any given small maximum diameter while preserving desired fiber length. That is, there always exist particles of associated impurities together with spicules of comparatively large diameter fiber in commercial asbestos spinning fiber mixes, and the yarn spun therefrom is characterized by attached or entangled bits of foreign material and unopened or apparently unopenable fibrous material.

It is an object of the present invention to substantially free asbestos from the aforesaid impurities and oversized particles of asbestos or other material normally occurring in or remaining in asbestos agglomerates, including mechanically fiberized or commercial mill fiber which may already have been subject to previously known refining methods, so as to enable production of asbestos products, especially from spinning grade length asbestos fibers of smooth, level character and general fineness, not accompanied by coarse oversized spots of harsh fiber or other foreign matter, whereby fabrics of felted, woven or extruded asbestos of greatly improved appearance and physical properties may be produced. Fibers of spinning grade length are those known as #1 and #2 crude, and the group of #3 grades of mill fibers, in accordance with Canadian chrysotile classification.

2

In general, I accomplish the objects of the present invention by first making a stable, aqueous dispersion of asbestos by means of an asbestos dispersing agent, as described in my co-pending application, Serial No. 66,552, filed December 21, 1948, now Patent No. 2,626,213, and then refine it by means of generally conventional screening or centrifuging apparatus.

The accompanying drawings diagrammatically illustrate means for segregating impurities and oversized material from the aforesaid stable, asbestos dispersion.

Fig. 1 diagrammatically illustrates an elevation, partly in section, of an arrangement employing a diaphragm or flat screen-type apparatus which may be employed for refining asbestos after the asbestos has been dispersed in accordance with my invention.

Fig. 2 is a plan view of the slotted screen plate employed in Fig. 1.

Fig. 3 is an elevation, partly in section, illustrating a screw feed strainer which may be employed for refining asbestos in accordance with my invention.

Fig. 4 is a front elevational view of a slotted strainer plate employed in the device of Fig. 3.

Fig. 5 is a sectional view of a ram extruder straining device which may be employed for refining dispersed asbestos in accordance with my invention.

Fig. 6 is a sectional view of a centrifugal separator provided with a slotted screen basket for refining dispersed asbestos in accordance with my invention.

Fig. 7 is a sectional view of a centrifugal refiner which also may be employed in accordance with my invention, and as a non-fully equivalent alternative for the apparatus shown in Fig. 1 when handling dilute, i. e. 0.1% to 1.0%, asbestos dispersions.

As more fully described in my aforesaid co-pending application, macroscopic bundles or agglomerates of asbestos (which terms are intended to include mechanically fiberized asbestos) are subjected to mild mechanical action, such as stirring or agitation such as, for example, in a vessel provided with vertical cylindrical bars rotating therein while immersed in water containing an asbestos dispersing agent. Paper beaters, Jordan engines, and the like attrition machines are highly undesirable where fiber length maintenance is important. The asbestos dispersing agents are organic detergent surface-active materials adsorbable on the asbestos and capable of forming an alkaline dispersion therewith, the

amount of detergent being in excess of that adsorbed on the asbestos and sufficient to form and preserve or maintain the dispersion in a stable manner. Typical examples of such dispersing agents are Aerosol OT (dioctyl sodium sulfosuccinate), sodium oleate, and others more fully particularized in my said co-pending application. Treatment of the asbestos in this manner causes separation, individualization, dissemination and unclothing of the asbestos fibers, and converts them to single fibers or fascicular fiber bundles instead of the predominantly clotted and tangled multiple fiber groups known to prior wet or dry asbestos practice. The fibers in such dispersion are in a lubricated, slippery, relatively slideable condition and composed predominantly of asbestos fibers of unit size, or "fibro-colloidal" diameter, that is, of a diameter of from about 200 to about 500 angstrom units.

The following is one example of a typical method for producing an asbestos dispersion in dilute condition suitable for subsequent refining: To 1000 gallons of water were added 312 pounds of 25% Aerosol OT in water and dissolved. Then 212 pounds of Canadian 3R spinning grade chrysotile asbestos were added, which on stirring produced a smooth slurry of 2½% asbestos concentration. This was further diluted by adding water slowly in the volume proportion of 9 parts of the 2½% slurry to 47 parts water. This produced a ¾% dispersion on mixing for four hours of the character previously described.

Treatment of the asbestos in this manner not only dispersed and individualized the asbestos fibers, but freed previously occluded and entangled non-fibrous associated impurities of the character previously described. By taking advantage of the jellylike water-holding characteristics of the opened mass, it may be strained through fine slotted screen plates such as are used in paper and pulp screening as illustrated in Fig. 1. The mass will even pass through a wire screen, say 10 to 20 mesh, but tends to tangle badly on such screen because two ends of the same fiber may pass through two different openings in the screen and thereby hang on the screen.

Thus, when refining dilute dispersions, such as of 0.1% to 1.0% by weight of asbestos, I have found that the diaphragm or flat screen type of apparatus of Fig. 1 is highly effective in not only removing impurities of a non-fibrous nature, but also larger spicules of picrolite, and clots or bundles of oversize or inadequately opened fibrous material.

Referring to Fig. 1 of the drawings, a ¾% asbestos dispersion, prepared in accordance with the foregoing example, was supplied from the stock chest 10 through line 11 and valve 12 to the flat bed screening device generally indicated as 13. The device 13 is a conventional type of paper-making screen comprising a flat bed of brass screen plates 14 with fine slots 9 cut vertically through the brass plates. These slots may be as narrow as from about .010 to about .015 inch and having a length of about 4 inches. These brass plates are mounted within an upwardly open chamber 15 which receives the dispersion from the stock chest 10, the refined dispersion passing through the slots in the screen to the lower chamber portion 16 and is delivered therefrom through the passage 17 to the flow box 18 and then transferred from the latter by means of the conduit 19, valve 20 and pump 21 to the screened stock chest 22. A vibrating flexible diaphragm 23 at the bottom of the closed chamber section 16 actuated

by the eccentrically mounted plunger 24 forces the slurry up and down through the slots in the screen plates, thereby keeping them open, screening being accomplished by a combination of gravity flow and suction. The tailings are removed from one end of the screen plate 14, either intermittently or continuously, for example, by the diagrammatically indicated reciprocal scraper means 25. These tailings, as previously indicated, comprise large spicules of unopened bits of harsh yellow fiber (picrolite), grains of magnetite, rock, clots of fiber, pieces of wood, etc., such impurities being found in comparatively large proportion even in commercially opened fiber for yarn making. Other devices embodying slotted screen plates may be used, as, for example, the Jonsson screen which operates with the screen plates flooded with the slurry and removes the tailings by a controlled vibratory motion which carries them up an inclined screen plate surface into an exit trough.

For asbestos dispersions of the foregoing nature, that is to say below 1% asbestos concentration, I may, as a non-fully equivalent alternative, employ a centrifugal refiner, as diagrammatically illustrated in Fig. 7, and which is of the type used in the paper industry, such as Erkensator or Bird Centrifiner, which operate on the principle of removing tailings from the outer portion of the centrifuged pulp and the refined slurries from the center portion of the centrifuged pulp. This, as illustrated in Fig. 7, such device comprises a rotatably mounted cylinder 26 supplied at one end through its axial conduit 27, the refined pulp being discharged from the axial conduit 28 and line 29. The heavier tailings are discharged from adjacent the periphery of the cylinder 26 through the outlet 30 and to the fixed chamber 31, wherefrom they are discharged from the outlet 32 of the latter. Another device in which the centrifugal effect is obtained by causing the slurry to swirl violently in a rifled tube with an accompanying pressure drop is also effective. This is the Dirtec made by Bird Machine Co.

For the refining of heavier slurries or dispersions, for example 30% and upwards asbestos content, it is possible to use a variation of a strainer of the type used for removing oversize particles from rubber compounds, particularly where the compounds are to be later extruded. This variation is illustrated in Fig. 3 and comprises a hopper 33 for reception of the stock to be strained and an elongated cylindrical chamber 34 enclosing the pressure feed screw 35 driven through gear 36. In place of a heavy wire screen backed up by a perforated plate employed in rubber practice, I employ a heavy plate 37 provided with fine longitudinal slots therein of a construction similar to that of the slotted plate 14, illustrated in Figs. 1 and 2 employed in papermakers' screen for screening pulp. The screw 35 in my strainer is longer and larger than that conventionally employed in rubber strainer practice because of the lower friction of a plastic asbestos dispersion of the indicated concentration, than that of rubber compounds. Although not shown, means may be provided for rapid removal of the slotted plate for cleaning.

For more fluid dispersions, say from 10 to 30% asbestos concentration, I may employ an apparatus such as that shown in Fig. 5 comprising a cylindrical chamber 38 provided with a hydraulic arm 39 and a slotted screen plate 40, similar to that of the plate 31 of Figs. 3 and 4. By this

means a semi-plastic mass of such concentration may be effectively forced through the screen plate 40 and suitably refined thereby.

For asbestos dispersions below 10% concentration, I may suitably employ a centrifugal basket-type refiner, as illustrated in Fig. 6. This comprises an outer cylindrical chamber 41 containing a basket 42 mounted for rotation therein by means of the shaft 43 and pulley 44. The peripheral wall of this basket 42 is provided with elongated narrow slots 45, similar to the slotted plates previously described. The dispersed asbestos to be refined is supplied from the conduit 46 to the interior of the rotatable basket 42 and then the refined material passes through the slots 45 into the outer chamber 41 and is discharged therefrom through the conduit 47. The interior surface of the basket 42 is kept free of tailings by means of the fixed scraper 48. In general, the slotted screens serve to remove spicules and clots and grains larger than the openings, although some finer impurities entangled in the tailings are also removed; the centrifugal separators remove substances of different gravity, particularly magnetite, sand, and dense unopened bits of fibrous rock.

The asbestos dispersion which free, or substantially free, of foreign materials or unopened aggregates of asbestos, and thus, being of a refined nature, is suitable for fabrication into many useful products, such as generally described in my aforementioned co-pending application. For example, the dilute slurries may be sheeted out on a paper-making machine; thin webs thereof may be converted into smooth, level, fine yarns in accordance with the co-pending application of Novak-Palm, Serial No. 90,238, filed April 28, 1948, now Patent No. 2,578,941, and plastic or semi-plastic slurries, either refined as such as hereinbefore described, or concentrated from the highly dilute slurries, may be employed for the manufacture of extruded products, such as, for example, extrusion about wires in accordance with my co-pending application, Serial No. 85,187, filed April 2, 1949.

Although I have shown and described several devices and arrangements of apparatus for refining my asbestos dispersions, it will be understood that other related and modified arrangements of apparatus may be employed within the scope of my invention.

I claim as my invention:

The method of refining chrysotile asbestos which comprises reducing chrysotile asbestos agglomerates of spinning grade length fibers to the form of a stable, aqueous, individualized, fibro-colloidal dispersion, by mixing with said agglomerates an aqueous liquid containing organic surface active detergent adsorbable on the asbestos and capable of forming an alkaline gelatinous dispersion therewith, and segregating from said colloidal dispersion oversize and relatively different density particle material by subjecting said dispersion to slotted screening and centrifugal separation.

References Cited in the file of this patent

UNITED STATES PATENTS

| Number    | Name             | Date           |
|-----------|------------------|----------------|
| 660,764   | Welch            | Oct. 30, 1900  |
| 1,091,899 | Shartle          | Mar. 31, 1914  |
| 1,684,365 | Dolbear          | Sept. 11, 1928 |
| 1,741,869 | Mett             | Dec. 31, 1929  |
| 1,750,725 | Miller           | Mar. 18, 1930  |
| 1,885,113 | Jenkins          | Nov. 1, 1932   |
| 1,887,726 | Weber            | Nov. 15, 1932  |
| 1,899,106 | Richter et al.   | Feb. 28, 1933  |
| 1,907,616 | Tucker           | May 9, 1933    |
| 2,060,685 | Murphy           | Nov. 10, 1936  |
| 2,068,219 | Badollet         | Jan. 19, 1937  |
| 2,217,005 | Clapp            | Oct. 8, 1940   |
| 2,220,386 | Badollet         | Nov. 5, 1940   |
| 2,225,100 | Clapp            | Dec. 17, 1940  |
| 2,265,936 | Cowles           | Dec. 9, 1941   |
| 2,312,545 | Haug             | Mar. 2, 1943   |
| 2,335,373 | Woodward         | Nov. 30, 1943  |
| 2,338,904 | Cowles           | Jan. 11, 1944  |
| 2,352,968 | Orton            | July 4, 1944   |
| 2,376,687 | Goldstein et al. | May 22, 1945   |
| 2,376,688 | Goldstein et al. | May 22, 1945   |
| 2,386,713 | Pharo            | Oct. 9, 1945   |
| 2,419,155 | Orton, Jr.       | Apr. 15, 1947  |
| 2,460,938 | Koehne           | Feb. 8, 1949   |
| 2,626,213 | Novak            | Jan. 20, 1953  |

FOREIGN PATENTS

| Number            | Country   | Date          |
|-------------------|-----------|---------------|
| 159,284           | Germany   | Mar. 17, 1905 |
| 13,412<br>of 1928 | Australia | Feb. 19, 1929 |